# EUROPEAN PATENT SPECIFICATION

(11) **EP 1 380 719 B1**
(45) Date of publication and mention of the grant of the patent: **14.12.2005**
(21) Application number: 03254110.4
(22) Date of filing: 27.06.2003
(51) Int. Cl.: E21B 10/56

(54) **Cutter and method of manufacture thereof**
Schneideinsatz und zugehöriges Herstellungsverfahren
Outil de coupe et procédé de fabrication de celui-ci

(30) Priority: 12.07.2002 US 64428
(43) Date of publication of application: 14.01.2004
(73) Proprietor: Camco International (UK) Limited, Stonehouse, Gloucestershire GL10 3RQ (GB)
(72) Inventor: Griffin, Nigel Dennis, Gloucestershire GL10 3UB (GB)
(74) Representative: Bailey, Richard Alan

(56) References cited:
- EP-A- 1 182 325
- GB-A- 2 335 682
- US-A- 5 492 188

## Description

This invention relates to a cutter, and to a method of manufacture thereof. The invention relates, in particular, to a cutter suitable for use on a drill bit for the formation of subterranean well bores. It will be appreciated that the cutter may alternatively be used in other applications.

One form of drill bit for use in the formation of subterranean wellbores comprises a bit body having a first end provided with a plurality of generally radially extending upstanding blades and a second end adapted to be secured to a drill string. Each of the blades carries a plurality of cutters. The cutters typically each comprise a tungsten carbide or other metallic substrate to which is bonded a layer of a superhard material, for example polycrystalline diamond. The substrate may be bonded directly to the bit body, or alternately may be bonded to a relatively long substrate which, in turn, is secured to the bit body.

In another form of drill bit, cutters are mounted upon rotatable cones mounted upon a bit body. Each cutter is typically manufactured by placing a sintered tungsten carbide substrate and diamond crystals into a container with a suitable binder catalyst material, and subjecting the container to high pressure, high temperature conditions such that the diamond crystals bond to one another and to the substrate.

A number of different designs of cutter are known, the different designs arising from, for example, the use of substrates of different shapes. In one example, the substrate includes an upstanding peripheral wall extending around most, but not all of the circumference of the substrate. A cutter manufactured using a substrate of this shape includes a polycrystalline diamond table which only extends to the periphery of the cutter at the region where the peripheral wall is absent as shown in Figures 1 and 2. It has been found that in cutters of this type there is a tendency for the polycrystalline diamond table to crack. This is thought to be as a result of hoop stresses.

A number of cutter designs provide the cutter with two or more cutting surfaces. This is achieved, in some designs, by providing two separate substrates, a first diamond layer located between the substrates and assecond, isolated diamond layer located upon the second substrate. This type of cutter is shown in US Patent No. 5,722,499 and US Patent No. 5, 667, 028. Another dessign includes separate diamond layers formed by providing grooves in the outer periphery of the substrate and introducing diamond crystals into the grooves prior to undertaking the high temperature high pressure process. Cutters of this type are illustrated in US Patent No. 5,979,578 and US Patent No. 5, 667, 028. It will be appreciated that, in these arrangements, two or more independent, isolated regions of polycrystalline diamond are formed.

The present invention provides a cutter with a reduced tendency for the polycrystalline diamond table to crack, and a method for manufacture of such a cutter.

EP 1182325 describes a cutter with a molybdenum layer encircling the diamond layer thereof. GB 2335682 and US 5492188 both describe arrangements having multi-part substrates, but in which only one of the substrate parts extends to the periphery of the cutter.

According to the present invention there is provided a method of manufacturing a cutter comprising assembling a first substrate component, a second substrate component and diamond crystals into a desired configuration, and subjecting the assembly to high temperature and high pressure conditions to cause the diamond crystals to bond to one another and to both the first and second substrate components to form a cutter having a single body of polycrystalline diamond, the first and second substrate components both extending to the periphery of the cutter and both being of the same material.

The first and second substrate components may be arranged to engage one another, or alternatively may be separated from one another by at least some of the diamond crystals prior to subjecting the assembly to high temperature, high pressure conditions.

The first and second substrate components are preferably of sintered tungsten carbide form. However, this need not be the case and other materials could be used. A binder catalyst material, for example cobalt, may be included in the assembly. Although cobalt is the preferred binder catalyst material, other iron group elements may be used, if desired. The binder catalyst material may be included in either of the first and second substrate components, or mixed with the diamond powder, or provided in any combination of these locations.

Also disclosed is a cutter with a single diamond table bonded both to first substrate component of circular cross-section and to a second substrate component of annular or part-annular form, the first and second substrates both extending to the periphery of the cutter and both being of the same material. At least one further substrate component, for example of annular or part-annular form, may additionally be provided.

According to another aspect of the invention there is provided a method of manufacturing a cutter comprising forming an assembly by locating a powdered substrate component material, diamond crystals and a first substrate component within a container in a desired configuration, and subjecting the assembly to high temperature and high pressure conditions to cause the powdered substrate component material to form a second substrate component and the diamond crystals to bond to one another and to both the first and second substrate components to form a cutter having a single body of polycrystalline diamond, the first and second substrate components extending to the periphery of the cutter and being of the same material as each other.

The powdered substrate component material is preferably powdered tungsten carbide. As mentioned hereinbefore, a binder catalyst material may be provided, for example mixed with the powdered substrate component material.

The configuration of the powdered substrate component material within the assembly may be such as to result in the formation of at least one additional substrate component. The second and/or additional substrate components may be of annular or part-annular form.

The invention also relates to a cutter manufactured using either of the methods described hereinbefore.

The invention will further be described, by way of example only, with reference to the accompanying drawings.
Figure 1 is a diagrammatic sectional view of a prior art cutter.
Figure 2 is an end view of the prior art cutter of Figure 1.
Figure 3 is a perspective view of a drill bit.
Figure 4 is a perspective view of an alternative drill bit.
Figures 5 and 6 are views similar to Figures 1 and 2 showing a cutter in accordance with an embodiment of the invention.
Figure 7 is a diagrammatic view illustrating part of the manufacturing operation.
Figures 8 to 25 are cross-sectional and side views of other embodiments.
Figure 26 is a view similar to Figure 7 illustrating an alternative manufacturing technique.

Referring now to Figure 3 there is shown a drill bit for use in the formation of subterranean wellbores. The drill bit comprises a bit body 10 having a first end 12 upon which a plurality of blades 14 are provided, the blades 14 upstanding from the first end 12 and extending in generally radial directions. The bit body 10 further includes a second end 16 adapted to permit the drill bit to be secured to the remainder of a drill string whereby the drill bit can be driven for rotation about its longitudinal axis 18. Each of the blades 14 is provided with a plurality of cutters 20, each of the cutters 20 being arranged to engage the formation being drilled using the drill bit, in use, such that the combination of rotation of the drill bit and the application of a load, in a generally axial direction, upon the drill bit causes the cutters to scrape the material from the formation. The drill bit further includes a plurality of nozzles 22 supplied with fluid and arranged such that, in use, fluid supplied through the nozzles 22 serves to clean the cutters and to carry the material removed by the cutters away from the drill bit.

As is common practice with drill bits of this type, the drill bit includes a gauge region 24. In the arrangement shown, the gauge region 24 is provided with a plurality of inserts 26 intended to enhance the ability of the drill bit to withstand wear of the gauge region.

Figure 4 illustrates an alternative type of drill bit. In the drill bit of Figure 4, the bit body 110 has an upper portion 116 which form legs 124 shaped to define mounting regions which in turn carry rotatable rollers 128 of generally conical form. Each of the rollers 128 is provided with a plurality of cutters 120. As with the drill bit illustrated in Figure 3, in use, the drill bit of Figure 4 is rotated about its axis 118. With the drill bit of Figure 4, such rotation causes the rollers 128 to rotate about their own axes, this movement causing the cutters 120 to engage and scrape against the formation being drilled to remove material therefrom which, as in the arrangement illustrated in Figure 3, is removed by the application of drilling fluid. Similar to the drill bit of figure 3, gauge inserts 126 are also provided.

Cutters 20, 120 may have various shapes and sizes as shown. However, for ease of understanding, the references and explanations for cutters 20 in this specification apply equally to cutters 120, as both types may be useful in both types of drill bits shown. The cutters 20, 120 may also be useful in numerous other type of down hole tools and other devices employing highly wear resistant cutting elements.

Figures 5 and 6 illustrate one of the cutters of the drill bits shown in Figures 3 and 4. The cutter 20 shown in Figure 5 comprises a first tungsten carbide substrate component 30 of generally cylindrical form, a second substrate component 32, also of tungsten carbide, and of part-annular form as shown in Figure 6, and a polycrystalline diamond table 34. The cutter 20 is manufactured by placing the second substrate component 32 into part of a suitable container 36, positioning powdered diamond crystals 34a in the region in which the table 34 of polycrystalline diamond is to be formed, and positioning the first substrate component 30 onto the second component 32 and diamond crystals 34a. The container 36 is then closed and sealed, as shown in Figure 7, the assembly then being subjected to high temperature, high pressure conditions to cause the diamond crystals 34a to bond to one another and to the first and second substrate components 30, 32. It will be appreciated that the formation of such bonds results in the production of the polycrystalline diamond table 34. In order for the table 34 of polycrystalline diamond to form, the assembly shown in Figure 7 may further include a quantity of a suitable binder catalyst material. Typically, the binder catalyst material takes the form of cobalt. However, a number of other materials could be used. In particular, any iron group element may be used as the binder catalyst material. The binder catalyst material may be introduced into the assembly by mixing the binder catalyst material with the diamond crystals 34a, or by incorporating the binder catalyst material into one or other, or both of the first and second substrate components 30, 32, or by including the binder catalyst material in the material of the container 36, or by a combination of these techniques. Where the binder catalyst material is included in the substrate components, it will be appreciated that it infiltrates into the diamond material during the high pressure high temperature operation.

After completion of the high temperature, high pressure sintering operation, the container 36 is removed and the cutter subjected to a suitable machining operation, if desired.

It will be appreciated that the cutter 20 manufactured using this technique and as shown in Figures 5 and 6 is similar in appearance to the known cutter shown in Figures 1 and 2. However, the use of the two-part substrate results in the application of significantly lower magnitude hoop stressing to the polycrystalline diamond table, the separate second substrate component 32 being more compliant than arrangements in which a single substrate is used, and as a result the risk of cracking of the polycrystalline diamond table is significantly reduced.

Although the technique described hereinbefore with reference to Figures 5, 6 and 7 can be used to produce a cutter 20 which is similar to that of Figures 1 and 2, the same technique may be used to manufacture a wide range of other cutter designs. A number of possible cutter designs are shown in Figures 8 to 19. In the arrangement illustrated in Figures 8 and 9, the first and second substrate components 30, 32 are spaced apart from one another by a part of the polycrystalline diamond table 34. It will be appreciated that a cutter of this type may be produced simply by positioning the second substrate component 32 within one part of the container 36, introducing the diamond crystals 34a into the container 36, the diamond crystals 34a extending over the second substrate component 32, and then introducing the first substrate component 30 so that diamond crystals 34a are located between the substrate components 30, 32. The application of high pressure, high temperature conditions to such an assembly will result in the production of a cutter 20 of the type shown in Figures 8 and 9.

Figures 10 and 11 illustrate a cutter 20 which is similar to that of Figures 8 and 9 but in which an additional, third substrate component 38 is located between the first and second substrate components 30, 32. In this arrangement, the polycrystalline diamond table 34 extends between the first and third substrate components 30, 38 and between the third and second substrate components 38, 32. The manufacturing process used in the formation of a cutter 20 of this type simply requires the introduction of the second substrate component 32 into the container 36, the application of diamond material into the container 36 covering the second substrate component 32, the introduction of the third substrate component 38 into the container 36, the application of more diamond material to cover the third substrate component 38, and finally the introduction of the first substrate component 30.

The arrangement shown in Figures 12 and 13 is similar to that of Figures 10 and 11 but includes a fourth substrate component 42. A further distinction between the arrangement of Figures 12 and 13 and that of Figures 10 and 11 is that no diamond material is provided between the various substrate components. It will be noted from Figures 11 and 13 that in each of these arrangements, the angular extent of the various part-annular substrate components are not equal resulting in the formation of steps in the polycrystalline diamond table 34. This need not be the case. The arrangement of Figures 10 and 11 further differs from that of Figures 12 and 13 in that, as shown in Figure 12, the various part-annular substrate components are of non-equal radial extent whereas in the arrangement shown in Figure 10, the second and third substrate components 32, 38 are of equal radial extent.

Turning to the arrangement shown in Figures 14 and 15, the second and fourth substrate components, 32, 42 are of equal radial extent and equal angular extent, the third substrate component 38 being of smaller radial and angular extent with the result that the polycrystalline diamond table 34 includes a radially extending projection 34b around part of its periphery.

The arrangement shown in Figures 16 and 17 is similar to that of Figure 8, but differs therefrom in that the second substrate component 32 is not located at the surface of the cutter, but rather is buried within the polycrystalline diamond table 34.

In each of the arrangements described hereinbefore, the first substrate component 30 is of generally cylindrical form having a flat surface to which the other substrate components and/or the polycrystalline diamond table 34 is bonded. This need not be the case, and Figures 18 and 19 illustrate an arrangement in which the surface of the first substrate component 30 is grooved. As a result, an arrangement is possible in which in some areas of the cutter 20, the second substrate component 32 rests directly upon the first substrate component 30, and in other regions thereof the second substrate component 32 is spaced from the first substrate component 30. In the regions where the second substrate component 32 is spaced from the first substrate component 30, as shown in Figure 19, then the polycrystalline diamond table 34 extends between the first and second substrate components, 30, 32.

In each of the arrangements described hereinbefore, it is important to note that the polycrystalline diamond table 34 is in the form of a single element, rather than taking the form of two or more separate components spaced apart and isolated from one another by a component of the substrate.

Although the cutters 20 described hereinbefore are suitable for use with drill bits of the type illustrated in Figure 3, it will be appreciated that by appropriate selection of the shape of the cutter, similar cutters may find application in drill bits of the type illustrated in Figure 4. A cutter 20 more applicable for use in a drill bit of the type illustrated in Figure 4 is shown in Figure 20.

The cutter 20 shown in Figure 20 comprises a first tungsten carbide substrate component 30 of generally cylindrical form but having a domed upper surface 50, in the orientation illustrated. A second substrate component 32 of annular form is positioned upon the first substrate component 30, the space within the second substrate component 32 containing a polycrystalline diamond table 34. The shapes of the second substrate component 32 and polycrystalline diamond table 34 are such as to define a domed surface 52. It will be appreciated that this type of cutter can be manufactured using a technique very similar to those described above.

It will be appreciated that a number of modifications can be made to the cutter of Figure 20, for example to change its shape so that the surface 52 is of, for example, generally conical form. Other variations include spacing the second substrate component 32 from the first substrate component 30, as shown in Figure 21, or including additional substrate components, as shown in Figure 22. The second and/or additional substrate components may be of annular or part-annular form. Where they are of curved, part-annular, form then depending upon their circumferential extent, two or more components may be provided at the same axial position as shown in Figure 23.

With cutters of the type used on drill bits of the type shown in Figure 4, it is common to provide one or more transition layers comprising a mixture of diamond and tungsten carbide between the tungsten carbide substrate and the polycrystalline diamond table. Such transition layers 54 may also be incorporated into the cutters shown in Figures 20 to 23. The second substrate component may be positioned upon the transition layer 54 or layers, for example as shown in Figure 24, or the transition layer 54 or layers may be at least partially encircled by the second substrate component, for example as shown in Figure 25.

In each of the arrangements described hereinbefore, the second and additional substrate components are of pre-sintered tungsten carbide form. It will be understood the other materials may be used, if desired. Where pre-sintered tungsten carbide substrate components are used, during the high pressure high temperature sintering operation the diamond will typically be compressed to a greater extent than the pre-sintered substrate components. This may result in, for example, a significant machining operation being required to produce a cutter having a flat or smooth face. It is thought that this effect may be reduced by modifying the manufacturing technique so that, instead of locating a pre-sintered second substrate component 32 with the container 36, and where appropriate instead of using pre-sintered third and fourth substrate components 38, 42, etc., a quantity of powdered tungsten carbide 56 is positioned in the container 36, as shown in Figure 26, in the areas in which the second substrate component 32, and where applicable the third and fourth substrate components 3 8, 42, etc., are required.

Once assembled, the application of the assembly to the high temperature, high pressure conditions will cause the second substrate component 32, and the third and fourth components 38, 42, etc., where applicable, to form as well as resulting in the formation of the polycrystalline diamond table and the bonding of the table to the first substrate component 30 and to the newly formed substrate components 32, 38, 42. As in the arrangements described hereinbefore, a binder catalyst material, typically cobalt, may be provided. The binder catalyst material may be mixed with the diamond powder, the tungsten carbide powder, the pre-sintered first substrate component 30, or in any combination of these locations.

During the manufacturing operation, the tungsten carbide forming the second substrate component 32 and, where appropriate, the additional substrate components, compresses at a rate similar to the powdered diamond with the result that a short, less complex machining operation may be required to produce a cutter with a generally flat or smooth surface.

It will be appreciated that this technique may be used in the manufacture of any of the cutters 20 described hereinbefore, or modifications thereto.

## Claims

1. A method of manufacturing a cutter comprising assembling a first substrate component (30), a second substrate component (32) and diamond crystals into a desired configuration, and subjecting the assembly to high temperature and high pressure conditions to cause the diamond crystals to bond to one another and to both the first and second substrate components (30, 32) to form a cutter having a single body of polycrystalline diamond (34), the first and second substrate components (30, 32) both extending to the periphery of the cutter and and **characterised in that** the first and second substrate components are both of the same material.

2. A method according to Claim 1, wherein the first and second substrate components (30, 32) engage one another.

3. A method according to Claim 1, wherein the first and second substrate components (30, 32) are spaced apart from one another, some of the diamond crystals being located between the first and second substrate components (30, 32).

4. A method according to Claim 1, further comprising assembling at least a third substrate component (38) with the first and second substrate components (30, 32) and diamond crystals.

5. A method according to Claim 1, further comprising locating the first and second substrate components (30, 32) and diamond crystals within a container prior to subjecting the assembly to high pressure, high temperature conditions.

6. A method according to Claim 1, further comprising including a binder catalyst material in the assembly.

7. A method according to Claim 6, wherein the binder catalyst material is an iron group element.

8. A method according to Claim 7, wherein the binder catalyst material is cobalt.

9. A method according to Claim 1, wherein the first substrate component (30) is generally cylindrical and the second substrate component (32) is of part-annular form.

10. A method according to Claim 1, wherein the first substrate component (30) is of grooved form.

11. A cutter comprising first and second substrate components (30, 32) and a single table of polycrystalline diamond (34) the table being bonded to both the first and second substrate components (30, 32), the first and second substrate components (30, 32) both extending to the periphery of the cutter and **characterised in that** the first and second substrate components are of the same material as each other.

12. A cutter according to Claim 11, further comprising at least one additional substrate component (38), the polycrystalline diamond table being bonded to the or each additional substrate component (38).

13. A cutter according to Claim 11, wherein the first substrate component (30) is of generally cylindrical form and the second substrate component (32) is of part-annular form.

14. A cutter according to Claim 11, wherein the first and second substrate components (30, 32) engage one another.

15. A cutter according to Claim 11, wherein the first and second substrate components (30, 32) are spaced apart from one another.

16. A cutter according to Claim 15, wherein the polycrystalline diamond table (34) extends between the first and second substrate components (30, 32).

17. A cutter according to Claim 11, wherein the first substrate component (30) is grooved.

18. A method of manufacturing a cutter comprising forming an assembly by locating a powdered substrate component material, diamond crystals and a first substrate component (30) within a container in a desired configuration, and subjecting the assembly to high temperature and high pressure conditions to cause the powdered substrate component material to form a second substrate component (32) and the diamond crystals to bond to one another and to both the first and second substrate components (30, 32) to form a cutter having a single body of polycrystalline diamond (34), the first and second substrate components (30, 32) extending to the periphery of the cutter and being of the same material as each other.

19. A method according to Claim 18, further comprising including a binder catalyst material in the assembly.

20. A method according to Claim 19, wherein the binder catalyst material is an iron group element.

21. A method according to Claim 20, wherein the binder catalyst material is cobalt.

22. A method according to Claim 18, wherein the powdered substrate component material is located to form an additional, third substrate component.

## Patentansprüche

1. Verfahren zum Herstellen eines Schneideinsatzes, das umfasst einen ersten Substratbestandteil (30), einen zweiten Substratbestandteil (32) und Diamantkristalle in eine gewünschte Konfiguration zusammenzubauen und die Baugruppe Bedingungen hoher Temperatur und hohen Drucks auszusetzen, um zu bewirken, daß sich die Diamantkristalle aneinander und an den ersten und den zweiten Substratbestandteil (30, 32) binden, um einen Schneideinsatz zu bilden, der einen einzigen Körper aus polykristallinem Diamanten (34) hat, wobei sich der erste und der zweite Substratbestandteil (30, 32) beide bis zum Umfang des Schneideinsatzes erstrecken, und **dadurch gekennzeichnet, daß** der erste und der zweite Substratbestandteil beide aus dem gleichen Material sind.

2. Verfahren nach Anspruch 1, wobei der erste und der zweite Substratbestandteil (30, 32) einander in Eingriff nehmen.

3. Verfahren nach Anspruch 1, wobei der erste und der zweite Substratbestandteil (30, 32) mit Zwischenraum zueinander angeordnet sind, wobei einige der Diamantkristalle zwischen dem ersten und dem zweiten Substratbestandteil (30, 32) angeordnet sind.

4. Verfahren nach Anspruch 1, das ferner umfasst, wenigstens einen dritten Substratbestandteil (38) mit dem ersten und dem zweiten Substratbestandteil (30, 32) und den Diamantkristallen zusammenzubauen.

5. Verfahren nach Anspruch 1, das ferner umfasst, den ersten und den zweiten Substratbestandteil (30, 32) und die Diamantkristalle innerhalb eines Behälters anzuordnen, bevor die Baugruppe Bedingungen hohen Drucks und hoher Temperatur ausgesetzt wird.

6. Verfahren nach Anspruch 1, das ferner umfasst, in die Baugruppe ein Katalysatorbindemittel einzuschließen.

7. Verfahren nach Anspruch 6, wobei das Katalysatorbindemittel ein Element der Eisengruppe ist.

8. Verfahren nach Anspruch 7, wobei das Katalysatorbindemittel Kobalt ist.

9. Verfahren nach Anspruch 1, wobei der erste Substratbestandteil (30) allgemein zylindrisch ist und der zweite Substratbestandteil (32) eine teilringförmige Gestalt hat.

10. Verfahren nach Anspruch 1, wobei der erste Substratbestandteil (30) eine gerillte Form hat.

11. Schneideinsatz, der einen ersten und einen zweiten Substratbestandteil (30, 32) und eine Einzeltafel aus polykristallinem Diamanten (34) umfasst, wobei die Tafel sowohl an den ersten als auch an den zweiten Substratbestandteil (30, 32) gebunden ist, wobei sich der erste und der zweite Substratbestandteil (30, 32) beide bis zum Umfang des Schneideinsatzes erstrecken, und **dadurch gekennzeichnet, daß** der erste und der zweite Substrabestandteil aus dem gleichen Material wie der jeweils andere sind.

12. Schneideinsatz nach Anspruch 11, der ferner wenigstens einen zusätzlichen Substratbestandteil (38) umfaßt, wobei die polykristalline Diamanttafel an den oder jeden zusätzlichen Substratbestandteil (38) gebunden ist.

13. Schneideinsatz nach Anspruch 11, wobei der erste Substratbestandteil (30) allgemein zylindrisch ist und der zweite Substratbestandteil (32) eine teilringförmige Gestalt hat.

14. Scheideinsatz nach Anspruch 11, wobei der erste und der zweite Substratbestandteil (30, 32) einander in Eingriff nehmen.

15. Schneideinsatz nach Anspruch 11, wobei der erste und der zweite Substratbestandteil (30, 32) mit Zwischenraum zueinander angeordnet sind.

16. Schneideinsatz nach Anspruch 15, wobei sich die polykristalline Diamanttafel (34) zwischen dem ersten und dem zweiten Substrarbestandteil (30, 32) erstreckt.

17. Schneideinsatz nach Anspruch 11, wobei der erste Substratbestandteil (30) gerillt ist.

18. Verfahren zum Herstellen eines Schneideinsatzes, das umfaßt, **dadurch** eine Baugruppe zu formen, daß ein pulverisiertes Substratbestandteilmaterial. Diamantkristalle und ein erster Substratbestandteil (30) in einer gewünschten Konfiguration innerhalb eines Behälters angeordnet werden, und die Baugruppe Bedingungen hoher Temperatur und hohen Drucks ansgesetzt wird, um zu bewirken, daß das pulverisierte Substratbestandteilmaterial einen zweiten Substratbestandteil (32) bildet und sich die Diamantkristalle aneinander und an den ersten und den zweiten Substratbestandteil (30) 32) binden, um einen Schneideinsatz zu bilden, der einen einzigen Körper aus polykristallinem Diamanten (34) hat, wobei sich der erste und der zweite Substratbestandteil (30, 32) bis zum Umfang des Schneideinsatzes erstrecken und aus dem gleichen Material wie der jeweils andere sind.

19. Verfahren nach Anspruch 18, das ferner umfaßt, in die Baugruppe ein Katalysatorbindemittel einzuschließen.

20. Verfahren nach Anspruch 19, wobei das Katalysatorbindemittel ein Element der Einsengruppe ist.

21. Verfahren nach Anspruch 20, wobei das Katalysatorbindemittel Kobalt ist.

22. Verfahren nach Anspruch 18, wobei das pulverisierte Substratbestandteilmaterial angeordnet wird, um einen zusätzlichen, dritten, Substratbestandteil zu bilden.

## Revendications

1. Procédé de fabrication d'un dispositif de coupe comprenant les étapes d'assemblage d'un premier composant de substrat (30), d'un deuxième composant de substrat (32) et de cristaux de diamant dans une configuration voulue, et d'exposition de l'assemblage à des conditions à température et pression élevées pour entraîner la liaison mutuelle des cristaux de diamant et la liaison aux premier et deuxième composants de substrat (30, 32) pour former un dispositif de coupe comportant un seul corps de diamant polycristallin (34), les premier et deuxième composants de substrat (30, 32) s'étendant tous les deux vers la périphérie du dispositif de coupe et **caractérisé en ce que** les premier et deuxième composants de substrat sont composés du même matériau.

2. Procédé selon la revendication 1, dans lequel les premier et deuxième composants de substrat (30,32) s'engagent l'un dans l'autre.

3. Procédé selon la revendication 1, dans lequel les premier et deuxième composants de substrat (30, 32) sont espacés l'un de l'autre, certains des cristaux de diamant étant agencés entre les premier et deuxième composants de substrat (30, 32).

4. Procédé selon la revende 1, comprenant en outre l'étape d'assemblage d'au moins un troisième composant de substrat (38) avec les premier et deuxième composants de substrat (30,32) et les cristaux de diamant.

5. Procédé selon la revendication 1, comprenant en outre l'étape de positionnement des premier et deuxième composants de substrat (30, 32) et des cristaux de diamant dans un récipient avant l'exposition de l'assemblage à des conditions de pression et température élevées.

6. Procédé selon la revendication 1, englobant en outre l'étape d'inclusion d'un matériau catalyseur de liaison dans l'assemblage.

7. Procédé selon la revendication 6, dans lequel le matériau catalyseur de liaison est constitué par un dispositif du groupe du fer.

8. Procédé selon la revendication 7, dans lequel le matériau catalyseur de liaison est constitué par du cobalt.

9. Procédé selon la revendication 1, dans lequel le premier composant de substrat (30) est généralement cylindrique, le deuxième composant de substrat (32) ayant une forme partiellement annulaire.

10. Procédé selon la revendication 1, dans lequel le premier composant de substrat (30) a une forme rainurée.

11. Dispositif de coupe comprenant des premier et deuxième composants de substrat (30, 32) et une seule table de diamant polycristallin (34), la table étant reliée aux premier et deuxième composants de substrat (30, 32), les premier et deuxième composants de substrat (30, 32) s'étendant tous les deux vers la périphérie du dispositif de coupe et **caractérisé en ce que** les premier et deuxième composants de substrat sont composés du même matériau.

12. Dispositif de coupe selon la revendication 11, comprenant en outre au moins un composant de substrat additionnel (38), la table de diamant polycristallin étant reliée au ou à chaque composant de substrat additionnel (38).

13. Dispositif de coupe selon la revendication 11, dans lequel le premier composant de substrat (30) a une forme généralement cylindrique, le deuxième composant de substrat (32) ayant une forme partiellement annulaire.

14. Dispositif de coupe selon la revendication 11, dans lequel les premier et deuxième composants de substrat (30, 32) s'engagent l'un dans l'autre.

15. Dispositif de coups selon la revendication 11, dans lequel les premier et deuxième composants de substrat (30,32) sont espacés l'un de l'autre.

16. Dispositif de coupe selon la revendication 15, dans lequel la table de diamant polycristallin (34) s'étend entre les premier et deuxième composants de substrat (30, 32).

17. Dispositif de coupe selon la revendication 11, dans lequel le premier composant de substrat (30) est rainuré.

18. Procédé de fabrication d'un dispositif de coupe comprenant les étapes de formation d'un assemblage en positionnant un matériau de composant de substrat sous forme de poudre, des cristaux de diamant et un premier composant de substrat (30) dans un récipeint dans une configuration voulue et d'exposition de l'assemblage à des conditions de température et pression élevées pour entraîner le matériau du composant de substrat sous forme de poudre à former un deuxième composant de substrat (32) et les cristaux de diamant à se lier les uns aux autres et aux premier et deuxième composants de substrat (30, 32) pour former un dispositif de coupe comportant un seul corps de diamant polycristallin (34), les premier et deuxième composants de substrat (30, 32) s'étendant vers la périphérie du dispositif de coupe et étant composés du même matériau.

19. Procédé selon la revendication 18, comprenant en outre retape d'inclusion d'un matériau catalyseur de liaison dans l'assemblage.

20. Procédé selon la revendication 19, dans lequel le matériau catalyseur de liaison est constitué par un dispositif du groupe du fer.

21. Procédé selon la revendication 20, dans lequel le matériau catalyseur de liaison est constitué par du cobalt.

22. Procédé selon la revendication 18, dans lequel le matériau du composant du substrat sous forme de poudre est destiné à former un troisième composant de substrat additionnel.
